

April 30, 1963

H. G. ROGERS  
PROCESS AND PRODUCT FOR FORMING COLOR  
IMAGES FROM COMPLETE DYES  
Filed Oct. 3, 1956

3,087,817



FIG. 1



FIG. 2



FIG. 3



FIG. 4

INVENTOR

*Howard G. Rogers*

BY *Brown and Mikula*  
*Stanley H. Morris*  
ATTORNEYS

## 1

3,087,817

**PROCESS AND PRODUCT FOR FORMING COLOR IMAGES FROM COMPLETE DYES**  
Howard G. Rogers, Weston, Mass., assignor to Polaroid Corporation, Cambridge, Mass., a corporation of DelawareFiled Oct. 3, 1956, Ser. No. 613,691  
39 Claims. (Cl. 96—29)

This invention relates to the art of photography and more particularly to novel processes for the formation of dye images and to film units and photographic products for use with such processes.

This application is a continuation-in-part of my pending application, Serial No. 358,012, filed May 28, 1953 (now U.S. Patent No. 2,774,668).

Objects of this invention are to provide processes for forming color images from complete dyes and involving the steps of providing, in a silver halide layer of a photosensitive element having a latent image therein, a solution of a dye and a silver halide developer of a character which has at least one oxidation product reactable with said dye to provide a reaction product having less mobility in the photosensitive element than the dye, whereby dye present in exposed areas may be immobilized, developing the latent image with said developer and acting upon dye in the exposed regions of the photosensitive layer with developer which is in oxidized condition whereby to substantially prevent the transfer of dye from the photosensitive element in proportion to the development of silver, while providing as a further result of silver development in the photosensitive layer an image-wise distribution comprising mobile dye and unreacted developer, and transferring at least part of said dye from said image-wise distribution to a print-receiving element located in superposed relation to the photosensitive element and depositing the transferred dye upon the print-receiving element and providing an image in terms of said dye; and also to provide processes such as those described which include the step of separating the photosensitive element and the print-receiving element by stripping said elements apart following the deposition of transferred dye on the print-receiving element.

Further objects of the invention are to provide processes of the character set forth wherein dye in solution in the photosensitive element is trapped or retained at least adjacent the exposed regions of a silver halide layer of said element by the reaction therewith of an oxidation product of a silver halide developer of a character capable of providing, upon the reduction of latent silver halide to silver, a substance which is reactable with said dye to provide a substantially immobile reaction product in the photosensitive element.

Still other objects of the invention are to provide processes of the nature described for forming color images from complete dyes wherein dye and unreacted developer from unexposed and less than completely exposed regions of a photosensitive element are transferred to a print-receiving element, as well as where the transfer of dye is effected, substantially to the exclusion of unreacted developer, to the print-receiving element; to provide processes utilizing procedures for keeping developer out of the print-receiving element and including the employment in the photosensitive element of a nondiffusing developer of the type having a large molecule whereby the developer is relatively immobile; to provide processes wherein dye which is reacted in the photosensitive element with the oxidation product of the developer is derived from a stratum of dye carried by the print-receiving element and in this regard especially to employ practices wherein a nondiffusing developer is incorporated in the

## 2

photosensitive element; and to provide processes of this general character which utilize a developer having an oxidation product reactable with dye to provide a substance having substantially the same color characteristics as said dye or a substance having color characteristics of a desired nature.

Yet other objects of the invention are to provide photographic products comprising a photosensitive element having a liquid-permeable portion including a silver halide layer, a print-receiving element positionable in superposed relation to the photosensitive element for receiving a transfer image, a container holding at least a liquid positioned for releasing its liquid between two layers of said product, and photographic processing materials, rendered effective by the release of liquid from the container, positioned in the product and including a dye which is soluble in said liquid and when dissolved therein is mobile in said photographic product, and also including a silver halide developer which is soluble in said liquid and is characterized by providing, upon the development of latent silver halide to silver, at least one oxidation product which is effective in preventing dye present in exposed regions of the photosensitive layer from transferring to the print-receiving element and which comprises a substance reactable with said dye to provide a reaction product which is less mobile in the photographic product than said dye.

Further objects of the invention are to provide photographic products of the character described having a developer characterized by providing an oxidation product reactable with said dye to provide as a reaction product a substance which is substantially immobile in said photosensitive element.

A further object of this invention is to provide processes of the nature described wherein the coupling function of the dye is insulated from the chromophoric system of said dye, and wherein a second chromophoric system, preferably of substantially the same color characteristics as the original chromophoric system, is formed by coupling with an oxidation product of the developer.

Still further objects of the invention are to provide photographic products of the character set forth which employ means for retaining the developer in the photosensitive element or for keeping the developer out of the print-receiving element and including the incorporation in the photosensitive element of a developer having a large molecule of a size sufficient to immobilize the developer in the photosensitive element, as well as to products wherein both the developer and the dye are translatable to the print-receiving element, and especially in this latter regard to products having a developer which provides an oxidation product reactable with dye to provide a substance having substantially the same color characteristics as the dye; and to provide photographic products such as those described which contain a dye mordant or an oxidizing agent in the print-receiving element and also such products wherein the dye is contained in the print-receiving element.

Yet further objects of the invention are to provide photosensitive elements having a support, at least one liquid-permeable layer on the support, silver halide distributed in a permeable layer of the element, a dye distributed in a permeable layer of the element and a silver halide developer distributed in a permeable layer of the element and wherein the dye is soluble in liquid and the developer is soluble in liquid and provides upon silver development at least one oxidation product effective in preventing dye present in exposed regions of the photosensitive layer from transferring from said element and comprising as said oxidation product a substance reactable with said dye to form a reaction product less mobile in said element than said dye; and to provide photosen-

sitive elements of the nature described wherein dye and developer of the kind set forth are contained in the same permeable layer or in individual permeable layers of said element including the permeable layer containing silver halide.

Other objects of the invention will in part be obvious and will in part appear hereinafter.

The invention accordingly comprises the several steps and the relation and order of one or more of such steps will respect to each of the others, and the products possessing the features, properties and the relation of elements which are exemplified in the following detailed disclosure, and the scope of the application of which will be indicated in the claims.

For a fuller understanding of the nature and objects of the invention, reference should be had to the following detailed description taken in connection with the accompanying drawing wherein:

FIGURE 1 is a diagrammatic side elevation of one embodiment of a film unit forming the subject of this invention and illustrates a product comprising a photosensitive element, a rupturable container and a print-receiving element;

FIG. 2 is a diagrammatic elevation of another embodiment of a photosensitive element forming the subject of this invention;

FIG. 3 is a diagrammatic elevation of still another embodiment of a photosensitive element forming the subject of this invention; and

FIG. 4 is a diagrammatic elevation of a further embodiment of a print-receiving element usable in carrying out the invention.

In general, the photographic processes and products disclosed herein, as in Patent No. 2,559,643, issued on July 10, 1951, to Edwin H. Land for Photographic Product and Process, are concerned with the treatment of a latent negative image in a photosensitive silver halide layer whereby to provide a dye positive image in or on another layer which comprises a print-receiving element.

In the just-mentioned Patent No. 2,559,643, there is disclosed a process adapted to be effected with a negative material in the form of a photosensitive element which includes a photosensitive silver halide layer and which has a conventional photographic coupler, for example a phenol, naphthol, pyrazolone or acetanilide type of coupler, and a silver halide secondary color-forming developer preferably incorporated in some permeable layer of the element. Para-phenylenediamine and derivatives thereof are classic examples of such developers. Other examples include aminophenol types of developers. A positive dye image of a latent image contained in the emulsion layer of the negative element is provided by spreading an alkaline liquid in contact with and between the photosensitive element and a permeable print-receiving element.

The spread liquid permeates into the negative element and developer dissolved in liquid within the element reduces the exposed silver halide of the latent image to metallic silver. Portions of the developer, which are oxidized as a result of silver development, react with the coupler in solution and form a dye image which is coextensive with the silver image. The unreacted developer and coupler in the remaining solution provide positive image-forming components which are transferred, by diffusion, from the photosensitive element to the print-receiving element and form thereon an imagewise distribution of unreacted developer and unreacted coupler which, upon oxidation of the unreacted developer, effect formation of the desired dye positive. Oxidation of the unreacted developer to cause coupling may be effected by an oxidizing agent incorporated in the print-receiving element or the coupling may be allowed to take place by serial oxidation of the developer after formation on the print-receiving element of the imagewise distribution

of the unreacted developer and unreacted coupler material.

Other related patents and applications which disclose the formation of dye images by coupling development and in a manner generally similar to that heretofore described are Patents Nos. 2,661,293 and 2,698,798, issued to Edwin H. Land on December 1, 1953, and January 4, 1955, respectively, the copending application of Edwin H. Land, Serial No. 448,441, filed August 9, 1954, now U.S. Patent No. 2,968,554, issued January 17, 1961, and also the copending application of Howard G. Rogers, Serial No. 577,711, now U.S. Patent No. 3,019,124, filed April 12, 1956.

Color development making use of conventional couplers and developers of a secondary color-forming type is subject to certain disadvantages. For example, many conventional couplers have different, and frequently, slow coupling rates. This difference in coupling rates makes it difficult to keep negative image-forming reactions separate in each light-sensitive elemental portion of a photosensitive element utilized in carrying out a one-step multicolor process, as well as obtaining sufficient density in short imbibition periods. Additionally, many dyes formed by coupling, especially so formed magenta and cyan dyes, have objectionable absorption characteristics and hence do not produce as accurate color renditions as desired. Furthermore, dyes formed by ordinary color development are, in general, sensitive to acid, and hence images comprised of these dyes may, in time, fade or change color when subjected to light or to acid gases present in the atmosphere.

The present invention is concerned with improvements in procedures and products utilized in the aforementioned applications and patent for the formation of dye images and especially for the formation of dye images by one-step photographic transfer processing. Accordingly, the invention will be described in connection with such transfer processes and products useful for carrying out the same, although, as will appear, the invention is not limited thereto.

The improvements herein are effected by the employment of complete dyes of a character soluble at least in alkaline solution and by the utilization of procedures and materials wherein dye which is substantially uniformly distributed in a photosensitive silver halide layer having a latent image therein will be immobilized or trapped or retained in exposed portions of the photosensitive layer upon development of the latent image to silver. As a result of development, there will be formed in the photosensitive layer a silver image and an image in terms of the material trapped or immobilized in the exposed regions of the photosensitive layer, while dye which is present in those regions of the photosensitive layer where no exposure or incomplete exposure and silver development have occurred is free for removal therefrom, as for example by transfer, at least in alkaline solution. Silver halide color developers which are soluble in alkaline solution are utilized with complete dyes in the carrying out of this invention. By this practice, use is made of a product resulting from the oxidation of a color developer by the development of a latent image in a silver halide layer to immobilize dye in the exposed and developed regions of the photo-sensitive layer.

Many dyes of the character with which this invention is concerned are reactable, as by coupling or other reaction, with an oxidation product of a color developer to provide a reaction product or substance which possesses less mobility in a photosensitive element than the original dye. Reactions of this nature occur when a para-phenylenediamine type of color developer which is employed in the development of a silver halide layer is utilized in conjunction with a complete dye. Similar reactions take place with aminophenol type developers.

The dyes employed are selected with a view towards

obtaining the greatest difference between the solubilities of the unreacted and reacted dye.

The invention also intends to make use of dyes which, while reacting with an oxidation product of a developer, provide a reaction substance which lacks the desired degree of immobility. For example, the reaction product or substance so formed may be only slightly less soluble than the original dye.

In instances where the substance produced by the reaction of a complete dye with an oxidation product of a conventional color developer lacks the desired immobility, a nondiffusing developer is employed which has a large molecule rendering it substantially immobile in the photosensitive element or is otherwise substantive to the emulsion medium. 4-amino-3-n-butoxydiethyl-aniline is an example of a nondiffusing color developer which has a long chain on its molecule. Another example is para-aminophenol to which a long carbon chain has been added. In nondiffusing developers of this type, the long chain will be retained on the developer molecule upon oxidation of the developer so that the product remaining after oxidation will still retain its immobility. Since the complete dye enters into a reaction with this product having the long chain on its molecule, the substance resulting from the reaction will also be retained in the photosensitive element.

It is also contemplated to employ nondiffusing developers in the processing of photosensitive elements comprising two or more differently sensitized emulsion elements, which elements may comprise a screen or a multi-layer arrangement. In such embodiments, it may be desirable in certain instances to employ different developing agents for each sensitized element.

Several mechanisms are thus presented by which a complete dye, which is at least soluble in alkaline solution, may be immobilized or retained in exposed regions of a photosensitive element while dye in unexposed regions of the element may be removed in solution, as for example by transfer. By way of recapitulation, by one mechanism an oxidation product of the developer reacts with the complete dye to form a substance which is less mobile in a permeable layer of the photosensitive element than the unreacted dye. By a second mechanism a nondiffusing developer having a molecule sufficiently large so that the developer is retained in the photosensitive element is utilized for immobilizing dye image components in the exposed regions of a photosensitive layer.

Common to these mechanisms is the fact that the color developer provides at least one substance upon its oxidation in the development of a latent image to silver which is capable of acting as an agent for immobilizing dye by reacting therewith so as to prevent its transfer from a photosensitive element. It may be here noted that experimental data leads to the belief that immobilization of dye image components in situ with the silver image developed by the developer is carried out primarily by the mechanisms just described and that any hardening of the carrier material of the photosensitive layer by reaction with the developer or some oxidation product thereof is a negligible factor in trapping and control of the dye.

The substance formed by the reaction of a complete dye and an oxidation product of the developer may possess color characteristics which are substantially the same as the unreacted dye or which are different from the unreacted dye. As will presently more fully appear, it is possible in carrying out a transfer process to form the transfer image either by the use of transferred dye which remains in unreacted condition or by the use of the product formed upon the reaction of the transferred dye with an oxidation product of the developer. The color of a substance formed by the reaction of an oxidation product of the developer and a complete dye becomes immaterial in instances where the complete dye is used

for transfer image formation and the reaction product is retained in the photosensitive element. In certain instances, it may be desirable to effect such a coupling reaction with the transferred dye, as for example, where the reaction product has a more desirable color.

A large number of complete dyes are available for the practice of this invention. Because of the wide choice of classes from which dyes may be selected as compared to the few available classes of couplers, as well as the ability of the invention to utilize a reacted dye molecule or an unreacted dye molecule, it is possible to form images of dyes having more highly accurate absorption characteristics, as well as images of dyes which are substantially stable. Additionally, in cases where a conventional type of color developer is to be immobilized in the photosensitive element, it is possible to achieve rates of development which are higher than those obtained with the para-phenylenediamine developers by the use of stronger color developers such as ring-substituted para-aminophenols as by one example wherein the ring substitution may be in the form of carbon chains. Furthermore, it is possible, because of the numerous usable dye classes and almost limitless number of dyes in them, to select dyes to carry out a multicolor process wherein the reaction rates of the different dyes will be similar in instances which utilize the reaction of an oxidation product of the developer and a complete dye for the purposes of immobilization.

The dyes which are useful in the processes of this invention are dyes possessing a coupling function. By a "coupling function" is meant a grouping in the dye molecule which enables the dye to couple, during development of the latent silver halide image, with an oxidation product of the silver halide developing agent. Typical coupling functions are (a) a phenolic hydroxyl group in a nucleus having the para positions free or occupied by radicals which split off during coupling, (b) a reactive methylene group, free or substituted by a radical which splits off during coupling such as an azo-linked group, and (c) an amino group on a ring in para position to an open position on the ring.

Among the classes from which suitable dyes are available, mention may be made of the monoazo, disazo, triphenyl methane, xanthane, thiazine and anthaquinone dyes. The field of dye materials is further extended by the employment of dye substances of the type which react with oxidized developer and which, in unreacted form, may be colorless in a particular environment, for example an acid environment, but upon change in the environment, for example to an alkaline environment, take on a color change. Dye substances of this type include indicator dyes, leuco dyes and carbinols of basic dyes.

Complete dyes of the character with which this invention is concerned are employable in a photosensitive element in the same manner as the conventional couplers previously mentioned, i.e., they are preferably incorporated in a permeable layer or stratum of the photosensitive element which may or may not contain other materials used in the photographic process, as for example silver halide and/or the developer. Dyes of the characteristics described and/or their reaction products should also be stable to light and to photographic solutions.

Dyes which are particularly suited for reaction with an oxidation product of a color developer are found in those dyes having an open position on a ring, which position is para to a hydroxyl or an amino group, or those dyes having a reactive methylene group. Many suitable dyes coming within this classification are found among the azo, pyrazolone and triphenyl methane dyes, specific examples of which comprise the following water- and alkali-soluble dyes such as Fast Fushine G (C.I. 29) for magenta; Fast Wool Yellow (C.I. 636) for yellow; Alphazurine 2G (C.I. 712) for cyan; and Polychrome

Blue-Black (C.I. 201) for black; as well as water-insoluble but alkali-soluble dyes, such as 1,5-dihydroxy naphthalene-4-azo benzene, for magenta; and Benzene Azo Resorcinol (C.I. 23) for yellow.

The substance formed by the reaction of a complete dye of the character described with the oxidation product of a standard type of color developer will usually possess color characteristics which are undesirably different from those of the unreacted dye as, for example, the grayish substance formed when the magenta dye, 1,5 dihydroxy naphthalene-4-azo benzene, is reacted with the oxidation product of a para-phenylenediamine type of developer. It therefore becomes necessary to utilize the unreacted dye molecule for image formation in transfer processing under circumstances wherein a reaction product of a color developer and a dye possesses an undesired color. However, it should be recognized that it is possible to use the reaction product for transfer image formation in instances where the oxidized developer reacts with the dye to give a reaction product which possesses a desired color, although such color may be different from that of the unreacted dye molecule.

Coupling dyes which possess a substituent replaceable by an oxidation product of a silver halide developing agent include dyes having open chain, reactive methylene groups having an azo substituent attached thereto, dyes having a heterocyclic system containing an azo-substituted methylene group and an adjacent carbonyl group as part of the ring structure, and dyes having an azo substituent attached to a phenolic nucleus in a position para to the hydroxyl group; see U.S. Patents 2,453,661, 2,455,169, 2,455,170 and 2,521,908. By suitable selection of compounds of this type or by the addition of solubilizing groups, one may have an initially soluble or mobile dye which may be rendered immobile by reaction with the oxidized developer. Thus, one may place the solubilizing groups, e.g., sulfo, on the displaceable azo substituent. In exposed areas, the coupling reaction will displace the azo substituent with its solubilizing groups and give an immobile product, while the dye in unexposed areas remains mobile and diffusible.

As further examples of complete dyes which react with the oxidation product of a silver halide developing agent to provide an immobile, nondiffusible reaction product, mention may be made of dyes containing a primary amino group, for example, anthraquinone and azo dyes containing primary amino groups. As an example of a silver halide developing agent having an oxidation product capable of reacting with a primary amino group, mention may be made of a developer such as pyrogallol.

Use of the unreacted dye molecule for image formation is made possible, when employing a para-phenylenediamine or other standard type of color developer, by preventing the reaction, on the print-receiving element, of dye and developer. In this regard, a number of varied practices are available.

By one practice for accomplishing this purpose, there is incorporated in the photosensitive element a developer which possesses a very low solubility in alkali but has good solubility in a high-boiling-point organic solvent. An example of such a developer is 4-amino-di-n-butylaniline. Procedures for carrying out this practice are known to the art and are set forth in Patent No. 2,478,400, as well as in the previously mentioned application Serial No. 448,441, now U.S. Patent No. 2,968,554. Due to the fact that the developer is of low solubility in alkaline solution, its mobility will be substantially restricted to the negative or photosensitive element.

Briefly stated, practices for incorporating a developer which is difficultly soluble in alkaline in a photosensitive layer are carried out by dissolving the free base of a standard developer in a high-boiling-point solvent such as tricresyl phosphate. The solution thus formed is then emulsified in a dilute gelatin solution containing an emulsi-

fying agent, as for example alkyl lauryl sulfate, and an appropriate amount of the emulsified product is added to a suitable quantity of a silver halide emulsion and is thoroughly mixed therewith. This procedure is also available for incorporating a dye in a silver halide emulsion which, along with the free base of the developer, may be dissolved in the aforementioned high-boiling-point solvent. However, since the dye is also soluble in alkali, it may be transferred in alkaline solution from the photosensitive element.

Alternatively, a relatively immobile or nondiffusing color developer, of the character previously mentioned, may be incorporated in the negative element as, for example, a developer having a long chain on its molecule such as 4-amino-3-n-butoxydiethylaniline. As a further alternative, the print-receiving element may include, as an image-receptive material, a plastic layer which is of a character displaying a greater affinity for dye than for developer or a preference for the penetration thereof by the dye over its penetration by developer. As an example of a receiving sheet material and a dye of these characteristics, mention may be made of partially hydrolyzed polyvinyl acetate and the previously mentioned magenta dye, 1,5 dihydroxy naphthalene-4-azo benzene.

As a still further means for controlling reaction of the dye in the print-receiving element, a strong reducing agent such as hydroquinone may be incorporated in the positive print-receiving element to prevent oxidation of any transferred developer and consequent coupling reaction.

These and similar practices are useful individually or in various combinations for the purpose of preventing the reaction of a transferred dye molecule with developer.

In addition to the well known types of color developers, as represented by the p-phenylene diamine type developers, it is also contemplated to employ  $\beta$ -aromatic sulfonhydrazide developing agents, the oxidation product of which will azo couple. Examples of such  $\beta$ -aromatic sulfonhydrazides are set forth in U.S. Patent No. 2,424,256. The developer may be appropriately substituted to render it nondiffusible or to so lower its mobility as to exclude its transfer to the image-receiving element. Coupling dyes especially suitable for use with developers of this type are dyes which are utilizable for azo coupling reactions.

In a further embodiment, it is contemplated to employ coupling dyes, the coupling function of which is insulated from the chromophoric system of said dye. By "insulated" is meant that the coupling function is separated from the chromophoric system by a link which prevents any system of conjugation or resonance from extending from the coupling function to the chromophoric system. Such coupling dyes would be immobilized in exposed areas in the manner described, and the transferred coupling dye would be free to couple with the oxidation product of the developing agent transferred from unexposed areas and oxidized after transfer. The coupling function and the developing agent are preferably so selected that the chromophoric system formed on coupling would have substantially the same color characteristics of the chromophoric system of the initial dye. This mechanism offers a method of increasing image dye density on the image-receiving element. As an illustration of an insulated coupling dye, mention may be made of dyes of the general formula:



wherein D is the residue of a dye, e.g., a cyan 1,4-bis-70 alkylamino-anthraquinone, n is 0 or an integer less than 5, and Q is the residue of a coupling function, e.g., a phenolic or naphtholic group which forms a cyan indo-phenol on coupling. Coupling of the transferred coupling dye may be effected by oxidizing the unreacted developing agent, e.g., by aerial oxidation or by the use

of an oxidizing agent present in or applied to the image-receiving element in a manner similar to that used with color couplers. The coupling dye and the oxidizing agent are preferably so selected as to avoid altering the chromophoric system of the dye in the course of the oxidation. It will be understood that such insulated coupling dyes may be employed without undergoing a coupling reaction on the image-receiving element. In addition, where such coupling is effected, the positive image may comprise both coupled and uncoupled coupling dye.

It is further contemplated to employ a coupling dye, the coupling function of which forms a substantially colorless reaction product with oxidized developer, i.e., the coupling reaction does not produce an additional chromophore.

In all embodiments of this invention, the dye forming the positive image contains the chromophore of the original dye. This feature will be readily apparent where one employs unreacted coupling dye or an insulated coupling dye to provide the positive image dye. Retention of the original chromophore in the positive image dye is also achieved, even though coupling is effected, by the use of coupling dyes the chromophore of which is not destroyed in the coupling reaction. An example of such a coupling dye is a naphthol having an azo group in the 2-position, color coupling being effected in the 4-position.

A further understanding of the invention will be gained from a consideration of products useful for carrying it into effect. In this regard, there is schematically shown in FIG. 1 a film unit making use of a negative sheet material or photosensitive element 10 comprising a support 11 of paper or film base material upon which there is mounted, in the order named, a layer 12 comprising a silver halide developer and a dye which is reactable with the oxidation product of the developer and a conventional photosensitive layer 14 of silver halide. The film unit of FIG. 1 also employs a positive sheet material or print-receiving element 15 comprising an image-receiving layer of opaque or transparent material which is liquid permeable and dyeable from alkaline solutions and which has been illustrated for purposes of simplicity as comprising a single sheet, for example, paper. However, the positive element 15 may comprise a support upon which at least one liquid-permeable and dyeable layer is mounted. It is also contemplated that the layer of liquid processing composition may serve as the image-receiving, i.e., dyeable, material under certain circumstances.

As shown in FIG. 1, the photosensitive element 10 and the print-receiving element 15, for the purpose of positive image formation, are adapted to be placed in superposed relation and are arranged so that the photosensitive layer or stratum 14 is next to the print-receiving element 15.

Also, in the film unit of FIG. 1 a rupturable container 16, adapted to carry an alkaline solution or liquid composition, is shown as positioned transversely of and adhered to the print-receiving element 15. If desired, the container 16 may be adhered to the photosensitive layer. Container 16 is of a length approximating the width of the film unit and is constructed to carry sufficient liquid to effect negative image formation in an exposed image area of the photosensitive layer 14 and positive image formation in the corresponding image area of the print-receiving element 15. In use, the container 16 is adapted to be positioned between the print-receiving element and the photosensitive element so that it will lie adjacent the edges of the corresponding image areas of these elements which are to be processed by the liquid contents of the container. When the film unit is of the roll film type, a plurality of containers are employed, one for each corresponding pair of successive image areas in the photosensitive and print-receiving elements. Details of such containers may be found in Patent No. 2,634,886, issued April 14, 1953, to Edwin H. Land for Collapsible Fluid Containers. Under certain circumstances, it may be desirable to apply the liquid processing composition prior

to exposure in accordance with the technique described in the copending application of Edwin H. Land, Serial No. 498,672, filed April 1, 1955.

In one embodiment, the layer 12 comprises a liquid-permeable carrier material in which is incorporated a dye of the character with which this invention is concerned and preferably a silver halide developer. The carrier material with the dye and/or developer therein is coated onto the support 11 to a thickness of about .0001 or .0002 inch. By another embodiment, the layer 12 may be formed of dye and developer dissolved in a volatile solvent or solvent mixture which is coated directly onto the support 11. The thickness of the layer 12 when formed in the last described manner will, of course, be infinitesimal. In any event, the layer 12 is penetrable by the liquid processing composition employed so that dye and/or developer contained therein may be placed in solution.

As will presently be pointed out, it is possible in this embodiment of the invention to locate the developer in the photosensitive layer 14 and, in certain instances, in solution in the liquid in the container 16. Also in this embodiment, the dye distributed in the layer 12 is preferably one of the water-insoluble but alkali-soluble dyes heretofore mentioned.

25 A suitable carrier material when layer 12 comprises a carrier in which dye and developer are distributed is one which will swell in hydroxide or alkaline liquids sufficiently to release dye and developer contained therein. Examples of carriers comprise gelatin, zein, polymethacrylic acid, shellac and cellulose acetate hydrogen phthalate, of which the latter may be named as preferred for most general purposes.

Where layer 12 comprises a carrier material in which dye and developer are distributed, one example of a composition for forming the layer is as follows:

1 gram 1,5 dihydroxy naphthalene-4-azo benzene  
1 gram 4-amino-3-n-butoxydiethylaniline  
4 grams cellulose acetate hydrogen phthalate  
80 cc. acetone  
20 cc. methanol  
1 cc. ethyl Cellosolve

In preparing this composition, the dye, developer and cellulose acetate hydrogen phthalate (the carrier material) are mixed together and dissolved in the solvent mixture provided by the acetone, methanol and ethyl Cellosolve. The composition so prepared is then coated onto the support 11.

50 The foregoing composition illustrates the use of a color developer which on oxidation will provide a reaction product of a color undesired for transfer image formation so that the dye in unreacted condition is intended to be employed to provide the transfer image. As may be noted, the developer in the foregoing composition is of the nondiffusing type so that it is substantially kept out of the print-receiving element. Additionally, a receiving sheet material such as partially hydrolyzed polyvinyl acetate may be used in the print-receiving element. Other practices such as those of the nature heretofore described are available for controlling developer transfer to avoid any coupling reaction on the image-receiving element.

55 Other dyes, for example of the same color or of a different color, such as a cyan or a yellow or a black dye, or combinations of differently colored dyes, may be substituted for the particular magenta dye of the foregoing formula.

The photosensitive silver halide layers used herein are provided by silver halide emulsions of conventional character which are coated onto the layer 12 after the latter has dried. The particular sensitivity range of each photosensitive layer, such as the layer 12, will be chosen to meet the particular requirement of use to which the photosensitive element will be put. These emulsions are conventionally coated onto the layer 14 or otherwise applied thereto to a thickness of from about .0002 to .0005 inch.

## 11

As heretofore mentioned, the image-receiving material of the positive element 15 includes any material dyeable from alkaline liquid. The positive element 15 may, as shown, comprise a single sheet of permeable material or it may comprise a support which carries a layer or a stratum of a permeable image-receiving material. An example of such is imbibition paper or baryta paper or conventional film base material upon which a permeable stratum is coated. As a further example, the print-receiving element may comprise a paper support subcoated with a substantially water-impermeable material such as a cellulose ester, i.e., cellulose nitrate, cellulose acetate and the like, and having a stratum of a permeable and dyeable material coated over the subcoat.

Image-receiving materials of a dyeable nature, in addition to those already named, include regenerated cellulose; polyvinyl alcohol; partially hydrolyzed polyvinyl acetate; sodium alginate; cellulose ethers, such as methyl cellulose or other cellulose derivatives such as sodium carboxymethyl cellulose or hydroxyethyl cellulose; papers; proteins, such as glue; carbohydrates, such as gums and starch; and mixtures of such materials where they are compatible. Polyvinyl alcohol may be named as a preferred image-receiving material for use with water-soluble dyes, especially with water-soluble dyes having sulfonate groups on the dye molecule. For water-insoluble dyes, a preferred image-receiving material is partially hydrolyzed polyvinyl acetate. Other preferred, especially for phenolic and naphtholic dyes, image-receiving materials are nylons, and preferably a nylon such as N-methoxymethyl polyhexamethylene adipamide, which is available under the trade name Nylon Type F8 from E. I. du Pont de Nemours & Co., Wilmington, Delaware.

The liquid processing composition employed in carrying out the invention comprises at least an aqueous alkaline liquid of sufficient alkalinity to permit the developer to perform its developing function and, in certain instances, may also have the developer dissolved therein. A viscosity-increasing compound constituting a film-forming material of the type which, when spread over a water-absorbent base, and dried will form a relatively firm, dimensionally stable film, is preferably included in the liquid processing composition to assist in carrying out the uniform spreading of the composition between the layers of the film unit. A suitable film-forming material is a high molecular weight polymer as, for example, a polymeric, water-soluble ether, inert to an alkaline solution, such as hydroxyethyl cellulose or sodium carboxymethyl cellulose. Liquid processing compositions of this nature are described in the previously mentioned patents and applications and in Patent No. 2,559,643. A suitable liquid processing composition comprises a mixture of 5 grams of sodium carboxymethyl cellulose, 3 grams of sodium hydroxide and 100 cc. of water. It is here pointed out that while sodium hydroxide is in general the preferred alkali used in the processing liquid, other alkaline materials may be employed, for example potassium or lithium hydroxide, sodium or potassium carbonate and diethylamine.

The incorporation of an oxidizing agent in the print-receiving element for the purpose of oxidizing unreacted developer permeated therein is disclosed in certain of the previously mentioned applications and in Patent No. 2,559,643. While the present invention will generally be practiced without the use of an oxidizing agent, it may be desirable in certain instances to utilize one, as where an insulated coupling dye is employed. For example, it may be preferred to form a transfer image of the reaction product of the complete dye and the oxidation product of a conventional color developer in instances where the reaction product has a suitable color. In such a case it may be desirable to include an oxidizing agent in the print-receiving element for the purpose of speeding up formation or increased density of the positive image.

As specific examples of suitable oxidizing agents, mention may be made of peroxy compounds such as sodium

## 12

or potassium perborate, certain dichromates such as ammonium dichromate, and compounds having polyvalent metallic elements in higher valent form such as copper, antimony, uranium, manganese, iron and cerium, wherein the metallic element is in higher valent form. Examples of these last-mentioned agents are cupric salts such as cupric sulfate. Another suitable oxidizing agent is benzoyl peroxide.

To build up greater density of image dye in the positive element, it may be preferable to have an efficient dye-precipitating mechanism included in the image-receiving sheet material. Consequently, it may be desirable to have a mordant included in the image-receiving sheet, as well as utilizing a print-receiving element having a layer or stratum which has an affinity for dye, such as a suitable plastic stratum. For this purpose, the print-receiving element itself may be formed of a conventional dye-transfer paper which contains a mordant. A suitable dye-transfer paper is commercially available from Eastman Kodak Company under the name of "Dye Transfer Double Weight F." As other examples, a print-receiving element may be provided with a gelatin layer containing a mordant such as nickelous sulfate or aluminum sulfate. Such a material may be used as the image-receiving stratum of the print-receiving element and is easily coated upon a support for the element. The use of a mordant in the print-receiving element is disclosed in the aforesaid Patent No. 2,559,643.

As another practice for providing a dye-precipitating mechanism in the print-receiving element, dyes may be chosen which form lakes with metal salts. Dyes of this character and metal salts usable for this purpose are well known to the art. Where the procedure of this type is utilized, metal salts such as chromium and/or barium salts are distributed throughout a permeable stratum of the print-receiving element in which the transfer image is provided.

In all products employed in the practice of the invention, it is preferable to expose the negative material or photosensitive element 10 from the emulsion side. It is therefore desirable to hold the photosensitive element 10 and positive sheet material 15 together at one end thereof by fastening means, not shown but comprising hinges, staples, or the like, in such manner that the photosensitive element 10 and the positive element 15 may be spread apart from their positions illustrated in FIG. 1. When the film unit is of the roll film type, the photosensitive element 10 and the positive sheet 15 are wound into separate rolls and the free ends of said rolls are connected together, in the manner described.

A camera apparatus suitable for processing roll film of the type just mentioned is provided by the Polaroid Land Camera Model 95 or similar camera structure, such for example as the camera forming the subject matter of Patent No. 2,435,717, issued February 10, 1948, to Edwin H. Land for Developing Camera Utilizing a Film, Another Sheet Material, and a Fluid Processing Agent. Camera apparatus of this character permits successive exposure of individual frames of the photosensitive element 10 from the emulsion side thereof, as well as individual processing of an exposed frame by bringing the exposed portion of the photosensitive element 10 in superposed relation with a portion of the print-receiving element 15 while drawing these portions of the film assembly between a pair of pressure rolls which rupture the container associated therewith and spread processing liquid between and in contact with the photosensitive element and the corresponding registered area of the print-receiving element.

Assuming that the film unit of FIG. 1 utilizes a layer 12 containing a magenta dye and a developer in accordance with the preceding formula, the processing of the unit for transfer image formation, following the exposure of the photosensitive element 10 to a desired subject, proceeds by rupturing container 16 and spreading the alkaline liquid processing composition between the photosensitive element and the print-receiving element.

## 13

The spread processing liquid migrates into the photosensitive layer 14 and the layer 12. During permeation into the layer 12, unreacted dye and unreacted developer contained in this layer are dissolved in the processing liquid and are transported in solution into the photosensitive layer 14.

Where the developer transported to the photosensitive layer 14 reacts with the exposed silver halide, it is oxidized as a function of the amount of silver halide reduced to silver and at least one oxidation product of the developer reacts with the dye adjacent the developing silver grains to form a reaction product. As previously noted, the product of the reaction of dye and the oxidation product of the developer is at least less mobile in the photosensitive element 10 than the dye itself.

For general purposes, since the developer is kept out of the print-receiving element, an excess of developer may be utilized in the photographic product. However, in instances where an oxidation product of the developer reacts with a coupling dye to provide a substance of desired color, developer is employed in a quantity controlled to avoid highlight stain in the transfer image. By this control, developer is utilized in a unit area of the layer, adapted to have the developer incorporated therein, in a quantity just sufficient to be completely oxidized by a fully developable or completely exposed silver halide portion of similar unit area.

In general, dye present in a dye-containing layer in a unit area thereof is preferably of a quantity just sufficient to be entirely reacted and immobilized by that amount of developer which is oxidized by the development of a completely exposed unit area of the photosensitive layer. This procedure avoids highlight stain in the transfer image. However, if the dye employed in the photosensitive element has a sufficiently low solubility rate, it is possible to use dye in excess of that just specified.

As intimated in the foregoing, processing of the nature described forms a substantially uniform distribution of dye and developer in the photosensitive layer 14 so that, upon development of silver, dye in the area of the highlights of the negative image is substantially exhausted by reason of its reaction with an oxidation product of the developer to provide a product which is at least less mobile in the negative sheet material than the dye itself.

As a further result of processing, in places in the negative material where unexposed silver halide grains are present or in places where exposure and subsequent development is less than complete, unoxidized or unreacted developer and dye are in an imagewise distribution proportional to silver development. Dye, and in certain instances developer, present in this imagewise distribution are both transportable, at least in part, by imbibition to the print-receiving element. However, the unreacted developer may be prevented from entering the print-receiving element by utilization of one of the precautions or practices previously described, such as the use of a non-diffusing developer, for example 4-amino-3-n-butoxydiethylaniline, or by the employment of a developer which is difficultly soluble in alkali, such as 4-amino-di-n-butyl-aniline. In all instances, the invention intends to transfer at least part of the dye to the print-receiving element to provide an image in terms of unreacted dye which is the reverse image of the latent image in the photosensitive element.

Following the formation on the print-receiving element of a reverse image of the latent image, the photosensitive element and the print-receiving element are separated, as by being stripped apart. In instances where the developer is retained in the photosensitive element 10 and/or is kept out of the print-receiving element 15, the reverse image on element 15 will comprise dye in unreacted condition. An advantage of this procedure resides in the simplification of processing and film unit construction by doing away with the need for an oxidation agent in the print-receiving element.

## 14

Where the developer is a standard color developer of the usual type such as a substituted para-phenylenediamine, an oxidizing agent such as disclosed in said Patent No. 2,559,643 is preferably included in the print-receiving element in instances where the reaction which takes place between the oxidation product of the standard color developer and the transferred dye provides a substance having the desired color characteristics. As pointed out, the use of an oxidizing agent, while not necessary, considerably speeds up reactions of this sort.

In the film unit of FIG. 1, a construction has been detailed wherein the developer and the complete dye are located in a stratum in back of the photosensitive stratum or between the photosensitive stratum and the support of the photosensitive element 10. This construction is generally preferred in carrying out a transfer process since it facilitates control of the reactants to the end of achieving substantially complete trapping or immobilization of dye and developer utilized in providing the negative image in the photosensitive element with consequent avoidance of highlight color in the positive.

However, the preferred construction is subject to considerable variation. For example, a layer or stratum containing the developer and/or unreacted dye may be located in front of the photosensitive layer. Also, the developer and the unreacted dye may be incorporated in individual strata of the photosensitive element, including the incorporation of one of these photographic materials in the photosensitive layer itself. Furthermore, in certain instances it is possible to omit the developer and/or dye from the photosensitive element and to include either or both in the alkaline liquid used for processing purposes. Also, the dye may be distributed in a stratum located on the side of the print-receiving element which is adapted to face the photosensitive element in instances where a nondiffusing type of developer is incorporated in the photosensitive element.

It has been previously pointed out that the photosensitive element 10 is designed preferably for use with water-insoluble but alkali-soluble dye. In general, many dyes will exert a desensitizing action on a silver halide emulsion if they become intimately mixed therewith, as for example by being imbibed into the emulsion from a solution of the dye. Desensitization may be of chemical character whereby the sensitivity of the silver halide is lowered. Also, desensitization may be of an optical nature, that is to say, dye which is intimately mixed with a silver halide emulsion will absorb actinic light intended for the exposure of the emulsion.

In forming the photosensitive element 10, the silver halide emulsion providing the layer 14 is coated onto the layer 12 after the latter has dried. It is possible for water or moisture in the wet emulsion to penetrate into the layer 12 although the carrier material for layer 12 is difficultly penetrable by water but is readily penetrated by alkaline solutions. If dye incorporated in the layer 12 is of a water-soluble nature, there is some likelihood of its entering into solution in water from the wet emulsion with subsequent migration into the photosensitive layer. In the photosensitive element 10, this possibility is avoided by utilizing a water-insoluble but alkali-soluble dye, for example, a dye such as the previously mentioned 1,5 dihydroxy naphthalene-4-azo benzene.

In instances where a dye which is soluble in water, as well as in alkali, is employed, a somewhat different type of photosensitive element is utilized. Such an element is shown in FIG. 2 and comprises a support 21 upon which is coated a layer 22 adapted to contain a water-soluble dye which is incorporated in a carrier material of the character previously described, for example, cellulose acetate hydrogen phthalate or gelatin. Coated upon the dye layer 22 is a barrier layer 23, comprising a carrier, such as cellulose acetate hydrogen phthalate, in which the developer is incorporated.

## 15

One composition suitable for forming a layer 22 comprises:

1 gram Fuschin (C.I. 29) (water-soluble dye)  
2 grams gelatin  
100 cc. water

An example of a composition suitable for providing the barrier layer 23 comprises:

4 grams cellulose acetate hydrogen phthalate  
2 grams 4-amino-3-n-butoxydiethylaniline  
80 cc. acetone  
20 cc. methanol  
1 cc. ethyl Cellosolve

After formation and drying of the layer 22, the layer 23 is applied thereon and, following the drying of the layer 23, the silver halide photosensitive layer 24 is coated on the layer 23. While water from the wet silver halide emulsion forming the photosensitive layer 24 may penetrate into the barrier layer 23, the barrier layer 23 may be made sufficiently thick so as to substantially prevent penetration of moisture from the wet emulsion of layer 24 into the layer 22 which contains the water-soluble dye. The photosensitive element 20 of FIG. 2 is susceptible to modification without change in its structural arrangement of layers. For example, the developer may be omitted from the layer 23 and included in the photosensitive layer 24.

The invention includes within its concept the incorporation of both the dye and the developer in layer 22 of the photosensitive element 20. In this instance, the barrier layer 23 will consist substantially only of the material which forms it.

The photosensitive element 20 is formed in a manner similar to the photosensitive element 10 and utilizes substantially similar materials for the purposes of construction. Likewise, the photosensitive element 20 is adapted to be used with a print-receiving element 15 of the nature disclosed in FIG. 1 and in a similar manner for providing, in the print-receiving element, a dye image which is the reverse image of a latent silver halide image formed in the photosensitive element 20 upon exposure thereof.

It has been further mentioned as an object of this invention to provide film units making use of a photosensitive element comprising a support having a photosensitive layer thereon in which both the dye and the developer are incorporated. Such a photosensitive element 30 is disclosed in FIG. 3 as comprising a support 31 having thereon a photosensitive layer 34 which incorporates silver halide, unreacted dye and a silver halide developer in a suitable carrier material, for example gelatin.

Practices for incorporating dye and a developer in a silver halide emulsion are similar to those well understood to the art for incorporating a coupler and a developer therein.

One nondiffusing developer for use with the photosensitive element 30 of FIG. 3 is the previously mentioned nondiffusing developer, 4-amino-3-n-butoxydiethylaniline. A composition comprising silver halide and 4-amino-3-n-butoxydiethylaniline of a nature suitable for providing the photosensitive layer 34 may be formed by dissolving the hydrochloride of the developer in water to which phosphoric acid approximately equal in amount to the developer has been added. The solution thus formed is added directly to the silver halide emulsion and the mixture is spread upon the support 31 to provide the photosensitive layer 34.

As previously set forth, there is a tendency among many dyes to effect emulsion desensitization when the dye is incorporated in a silver halide emulsion. Preferably, the invention utilizes a dye of a nature which exerts a minimum chemical and/or physical desensitizing action on a silver halide emulsion. Preferably, also, the dye employed is of a water-insoluble nature whereby to limit its intimate mixture with a silver halide emulsion to the end

## 16

of avoiding possible optical desensitization. An example of water-insoluble dye is the previously mentioned 1,5 dihydroxy naphthalene-4-azo benzene which may be mixed with a silver halide emulsion from a solution of the dye in acetone and methanol.

Furthermore, desensitization by dye in the emulsion may be avoided by encasing the dye in particles comprised of hardened gelatin and by distributing the dye-containing particles throughout the silver halide emulsion. These dye-containing particles may be formed by procedures similar to those taught in U.S. Patent No. 2,618,553. In place of hardened gelatin, the dye may be incorporated in particles of a material which is difficultly penetrable by water but is readily penetrated by alkaline solutions such, for example, as the cellulose acetate hydrogen phthalate, already mentioned, or similar materials. Colored dye materials which are incorporated in a photosensitive layer preferably have a particle size which is greater than the particle size of the silver halide grains whereby to lower the covering power of the dye to permit photographic exposure of the photosensitive layer to its full thickness.

Mention has been made of compounds in the nature of dyes which are substantially colorless in a particular environment but become colored when this environment is changed. Such compounds include indicator dyes, leuco dyes and carbinols of basic dyes. Dye substances of this nature should possess the properties heretofore enumerated as requisites for carrying out the purposes of this invention and, in addition, should preferably be colorless or yellow or slightly so in a neutral or acid environment. For example, indicator dyes such as 2,5-dinitrophenol, quinaldine red and quinoline blue have, respectively, a yellow, a red and a blue color at a relatively high pH but are substantially colorless in a neutral or acid environment.

Such dye substances as those capable of assuming a color change are especially adapted for use with a photosensitive element having a layer of silver halide in which the dye and the developer are incorporated as, for example, the photosensitive element 30 of FIG. 3. Since dye substances of this nature are utilized in a photosensitive element in their colorless form, it is possible to increase the concentration of the dye substances in the element without having any effect upon the satisfactory exposure of the photosensitive layer. Preferably, the dye of this nature is colorless at a pH of about 7. To provide an acid environment in the photosensitive layer, a suitable acid such as an appropriate amount of phosphoric acid may be added to the photosensitive emulsion. Alkali contained in the processing liquid will, in general, supply the alkaline environment needed for creating the desired color change in the dye substance. If dye substances of the nature under discussion exert a desensitizing effect upon the silver halide, practices such as those described may be utilized to restrain desensitization.

When a dye substance which is colorless in a neutral or acid environment is utilized in a photosensitive element such as the element 30, the portions of said substance which are employed to provide the positive image are transferred to the print-receiving element in unreacted form. One of the practices previously pointed out for restraining transfer of unreacted developer to the print-receiving element is utilized. The processing of the photosensitive element 30 is carried out in a manner similar to that heretofore detailed. In the case of some dye substances which change color according to their environment, it may be desirable to incorporate alkali, for example sodium carbonate, in the print-receiving element. Also, in the case of leuco dyes and carbinols of basic dyes, it may also be desirable to include an oxidizing agent in the print-receiving element for the purpose of speeding up the color change. Both of the latter-mentioned practices are included within the scope of the present invention.

The photosensitive element 30 is especially adapted for use with the embodiment of the invention wherein a photosensitive element has a nondiffusing developer incorporated in the photosensitive layer thereof and such an element may be utilized with a print-receiving element 45, shown in FIG. 4, which carries a stratum 47 of dye coated on the side thereof which is adapted to face the photosensitive element when processed. A dye stratum 47 is provided by incorporating the dye in a volatile solvent, for example 1 gram of dye in 100 cc. of acetone, and by coating the solution onto the surface of the print-receiving element 45. Print-receiving element 45 comprises any of the embodiments thereof heretofore specifically discussed. As another practice, the dye utilized may be incorporated in a carrier material, such as one of those already described, for coating in a thin layer upon the print-receiving element. In this embodiment, the photosensitive layer is prepared in the manner described from a composition comprising a silver halide emulsion to which has been added a solution of the hydrochloride of the developer in water and phosphoric acid.

In the embodiment of the invention utilizing a print-receiving element 45, a dye-precipitating mechanism is provided by the oxidation product of the nondiffusing developer incorporated in the photosensitive layer. Liquid spread between the photosensitive element and the print-receiving element is absorbed into both of these elements. In the photosensitive element, developer in solution in the absorbed liquid develops latent image therein and its oxidation product attracts dye placed in solution by the liquid in contact with the print-receiving element to cause liquid containing dye in solution to migrate into the photosensitive element in the exposed regions of the photosensitive layer where it is acted on by the oxidation product of the developer and becomes substantially immobilized or trapped in the photosensitive element. On the other hand, dye which may migrate into the photosensitive element but is not acted upon by the oxidation product of the developer is available in the usual manner for formation, on the print-receiving element, of a dye image which is the reverse of the latent image formed in the photosensitive element.

In cases where a photosensitive element is employed in which dye is incorporated, it is possible to make two or more transfer prints from the photosensitive element. This may be accomplished by utilizing a dye which is slowly soluble in alkaline solution and by employing a quantity of this dye in the photosensitive element which is in excess of that needed to provide a transfer print. Due to the fact that the dye used in this procedure is in excess of that required to provide a transfer print and because of its slow solubility rate, a quantity of this dye at least sufficient for a second transfer print remains in the processed photosensitive element. A second transfer print may be obtained by pressing the photosensitive element against an unused print-receiving element into which has been permeated a solvent for the dye. When sodium hydroxide is the alkali added to the liquid employed for processing the latent image, the dye in the photosensitive element will, in most instances, be converted to its sodium salt when in solution in the liquid. In general, the sodium salts of dyes are water soluble so that water may be employed as the liquid or solvent for effecting the second transfer of dye although, if necessary, an alkaline solution may be utilized.

Additionally, a photosensitive element such as the element 30 is useful in carrying out practices of this invention wherein the dye and/or the developer are included in the processing liquid such, for example, as in a container 16, although as heretofore pointed out it is usually preferable to incorporate both the dye and the developer in the photosensitive element.

Modifications of the film structure, in addition to those already discussed, are included within the scope of the

invention. For example, either the photosensitive element 10 or the photosensitive element 20 is useful for carrying out the invention when the developer is omitted from the element and is included in the processing liquid as in the container 16 shown in FIG. 1. The photosensitive element 10 is also available for practices wherein the developer is incorporated in the layer 12 thereof and dye is in solution in the processing liquid in container 16. Other modifications of the photosensitive elements 10 are possible. For example, either of the photosensitive elements 10 or 20 may include between the respective bases and the photosensitive layers thereof an additional liquid-permeable layer. In such event, developer may be distributed throughout such an additional layer and dye 15 may be distributed throughout the layer 12 or 22, or this procedure may be reversed. Also, as has been indicated, both the dye and the developer may be incorporated in the layer 22 of the photosensitive element 20.

The invention also contemplates the modification of 20 dyes to the end of improving their characteristics for use in the processes described herein. For example, a dye which has good characteristics as to color may not have the preferred characteristics for undergoing immobilization in a photosensitive element. It is possible to suitably 25 modify the dye to improve its overall characteristics. For example, 1,5 dihydroxy naphthalene-4-azo benzene provides much higher contrast images with a conventional color developer than its commercially available form which has sulfonate groups added thereto. Such 30 groups are solubilizing so that if a dye is too soluble and transfers too fast, it can be appropriately modified by omitting these solubilizing groups or by adding carbon chains of suitable lengths to the dye molecule.

Furthermore, a dye may be modified in other ways. 35 For example, if the dye does not couple efficiently with the color developer employed, it may be modified by condensation with a coupling function, e.g., a phenol or naphthol preferably having a chloro group para to the OH group of the phenol, and in such a way that there is no 40 conjugation between the new coupling function and the original dye, i.e., the coupling function is insulated, or, if the color of the original dye has changed, this change is in a desired direction. As a further illustration it may be noted that it is, in general, most convenient if the dye 45 is insoluble in water but is soluble in alkali. To decrease the solubility of such a dye in water, sulfonate groups thereon may be replaced with carboxy or sulfonamido groups. Generally, replacement of the sulfonate groups in this instance is preferred because omission of the sulfonate groups without replacement may deleteriously affect the stability of the dye.

It is particularly pointed out that practice of the invention is not limited to the use of cyan, magenta or yellow images. For example, dye positive images of a color other than those just mentioned are obtainable when several dyes, rather than a single dye, are employed in the photosensitive layer. The result of such an expedient is to give a positive image different from each of the individual dyes that are utilized for image formation. Thus, it 55 is possible to form black and white dye positive images by the use of suitably colored dyes in appropriate quantities which, when added together, give black.

While the present invention is particularly suited for the formation of colored images, it is to be especially observed that practices herein are also utilizable for the formation of black and white positive images by the use of a mixture of dyes as just described or by the use of a single dye which is black such as, for example, any one of the black dyes heretofore mentioned. Additionally, the use 60 of a black dye or a mixture of dyes which together provide black may be utilized for forming a black component in a multicolor picture.

The present invention finds particular utility in the field of color photography and, in addition to providing for the formation of monochromatic images of a single

color, is useful in providing multi-color images. For example, the practices set forth herein may be used to provide the light-sensitive elemental portions in a multi-color photo-sensitive element of the type set forth in the previously mentioned application Serial No. 448,441 (U.S. Patent No. 2,968,554) and also in my previously mentioned application Serial No. 358,011 (U.S. Patent No. 2,774,668). Such multicolor photosensitive elements are processed in the manner described in the just-mentioned applications for providing in one step a multicolor image on a print-receiving element.

Additionally, two or more transparent print-receiving layers, each containing an individual color component image of a multicolor image, may be assembled in superposed and registered relation on a common support in a manner well understood by the art whereby to provide the desired multicolor image.

As another example, the invention is adapted for multicolor work carried out with special film units wherein two or more appropriately sensitized photosensitive elements are associated with a like number of print-receiving elements in a manner similar to that set forth in Patent No. 2,647,049, issued to Edwin H. Land on July 28, 1953. Also, as shown in the last-mentioned patent, a plurality of color component images may be formed in the same print-receiving element by successively bringing the print-receiving element into registered contact with individual negative elements, each of which latter contains a negative latent image representative of a positive color component image to be formed in the print-receiving element.

The inventive concepts of this invention are also utilizable in connection with the integral multilayer photosensitive elements disclosed and claimed in the copending application of Edwin H. Land and Howard G. Rogers, Serial No. 565,135, filed February 13, 1956.

Furthermore, the invention is useful for copying purposes from separation positives with any of the types of film units described. Of course, when the invention is used in the production of photographic originals, the spectral sensitivity of the different emulsion layers must be suitably chosen. For instance, instead of using a blue-sensitive emulsion, a panchromatic or a specially red sensitized emulsion is employed for producing a cyan positive image. However, for copy work from separation positives, this is obviously unnecessary.

Also, as has been intimated, photosensitive elements of this invention are available for color image formation therein, such, for example, as a master negative image. In this regard, a photosensitive element containing a dye and a silver halide developer of the character described is exposed to a suitable subject, and the photosensitive element is then permeated with the usual alkaline liquid. The result of permeation of the alkaline liquid into the photosensitive element is to develop latent image therein to silver and provide a colored substance which is in situ with the silver image and is less mobile in the element than dye, this colored substance comprising the reaction product of dye in the photosensitive layer and an oxidation product of the developer.

As the result of development there is also provided in the photosensitive element an imagewise distribution of dye and unreacted developer in the unexposed regions of the photosensitive element which is removable, as for example by washing, from the element. Following the removal of dye and developer, there remains in the photosensitive layer a silver image and a color image comprising the relatively immobile colored substance in situ with the silver image. The silver image may then be removed by the use of conventional silver bleaches which will not harm the substance providing the colored image, for example a bleach such as a mixture of a sodium or potassium halide and potassium ferri-cyanide. Prior or subsequent to bleaching, the photosensitive layer may be fixed in conventional manner. If the developer, because of its low mobility, is difficult to wash out of the photosensitive

element, it is possible to effect its deactivation by appropriately acidifying it.

The inventive concepts herein set forth may be readily distinguished from the diffusion-transfer reversal color processes set forth in the previously mentioned Land Patent No. 2,559,643. In the processes of that patent, unreacted developer and unreacted color coupler are transferred to the image-receiving material and are oxidized and coupled to provide the dye image. The couplers disclosed in that patent are colorless or substantially colorless, and in no event can be considered to be dyes. The coupling reaction to provide the image dye is an essential feature of that process, and the color of the image dye is completely different from that of the coupler, even if the coupler were colored. The processes herein disclosed preferably utilize the unreacted coupling dye as the image dye. A coupling reaction on the image-receiving element between oxidized developer and a coupling dye is effected only in the case of an insulated coupling dye or to obtain a dye of a more desirable color. In any event, however, the positive image dyes of this invention still contain the chromophore of the unreacted dye, as contrasted with the fact that the chromophore of a colored color coupler is always destroyed on coupling.

While a liquid container 16, which has been illustrated with the film units of this invention, provides a convenient means for spreading a liquid composition between layers of a film unit whereby to permit the processing to be carried out within a camera apparatus, the practices of this invention may be otherwise effected. For example, a photosensitive layer, after exposure in suitable apparatus and while preventing further exposure thereof to actinic light, may be removed from such apparatus and permeated with the liquid processing composition as by coating the composition on the photosensitive layer or otherwise wetting the layer with the composition, following which the permeated layer, still without exposure to actinic light, is brought into contact with a print-receiving element for image formation in the manner heretofore described.

It is also to be kept in mind that the invention may be successfully practiced without the use of a film-forming material in the liquid processing reagent. As an illustration, with this latter expedient, a nonviscous processing composition is particularly applicable and may be applied to the negative material by imbibition or coating practices and may be similarly applied to the print-receiving element before the latter and the negative material are brought into superposed relation or contact for carrying out the transfer of positive image-forming components.

As used herein, the expression "developer" is intended to refer to silver halide developing agents which, as well known in the art, are compounds which develop a latent image contained in an exposed silver halide emulsion. The expression "color developer" is intended to refer to silver halide developing agents which provide an oxidation product upon the development of exposed silver halide, which oxidation product is capable of coupling with a color coupler.

Since certain changes may be made in the above products and processes without departing from the scope of the invention herein involved, it is intended that all matter contained in the above description or shown in the accompanying drawing shall be interpreted as illustrative and not in a limiting sense.

What is claimed is:

1. A process of forming images in color which comprises providing in a photosensitive element, including an exposed photosensitive silver halide emulsion having a latent image therein, a substantially uniform distribution, in said emulsion of a silver halide developing agent and a dye which possesses a coupling function capable of coupling with the oxidation product of said silver halide developing agent, said dye when dissolved in the processing liquid being mobile in said photosensitive element and said developing agent being characterized by providing,

21

upon the development of said latent image to silver, an oxidation product reactable with said dye to provide a reaction product less mobile in said photosensitive element than said dye; developing said latent image to silver and immobilizing said dye in the exposed regions of said emulsion by reaction with said oxidation product of said developing agent to substantially prevent the transfer of dye from said exposed regions of said emulsion while providing in unexposed regions of said emulsion an image-wise distribution comprising mobile dye; and transferring from unexposed regions of said emulsion, by imbibition, at least part of said image-wise distribution of mobile dye to a superposed print-receiving material to provide a positive dye image having substantially the same color as said mobile dye, said transfer of mobile dye being effected to the substantial exclusion of said less mobile reaction product.

2. The process of forming images in color as defined in claim 1 wherein the print-receiving material and the photosensitive element are separated from superposed relationship at some stage of said process after the image-wise distribution of mobile dye has been transferred from said photosensitive element to said print-receiving material.

3. The process of forming images in color as defined in claim 1 wherein said image-wise distribution of mobile dye is transferred to said image-receiving material substantially to the exclusion of transfer to said image-receiving material of unreacted developing agent.

4. The process of forming images in color as defined in claim 1 wherein unreacted developing agent is transferred from unexposed areas and oxidized, and the oxidation product of said developing agent is coupled with said transferred mobile dye.

5. The process of forming images in color which comprises spreading a liquid in a layer between and in contact with a photosensitive element comprising an exposed silver halide emulsion having a latent image therein and a print-receiving element comprising an image-receiving material; absorbing said liquid into said photosensitive element including said emulsion and providing in said emulsion a substantially uniform distribution of a silver halide developing agent and a dye which possesses a coupling function capable of coupling with the oxidation product of said silver halide developing agent, said dye when dissolved in said liquid being mobile in said photosensitive element and said developing agent being characterized by providing upon the development of said latent image to silver an oxidation product reactable with said dye to provide a reaction product which is less mobile in said photosensitive element than said dye; developing said latent image to silver with said developing agent and immobilizing dye in the exposed regions of said emulsion by reaction with said oxidation product of said developing agent to substantially prevent the transfer of dye from said exposed regions while providing in unexposed regions of said emulsion an image-wise distribution comprising mobile dye and unreacted developing agent; and transferring from said unexposed regions of said emulsion, by imbibition, at least part of said image-wise distribution of said mobile dye to said print-receiving element in superposed relation with said photosensitive element to impart to said image-receiving material an image having substantially the same color as said mobile dye, said transfer of mobile dye being to the substantial exclusion of said less mobile reaction product, said development and said transfer being effected by the application of a single liquid.

6. The process of forming images in color as defined in claim 5 wherein said image-wise distribution of mobile dye is transferred substantially to the exclusion of transfer to said image-receiving material of said unreacted developing agent.

7. The process of forming images in color as defined in claim 5 wherein said unreacted developing agent is

22

transferred to said image-receiving element, oxidized and coupled with said mobile dye.

8. The process of forming images in color as defined in claim 5 wherein the print-receiving element and the photosensitive element are separated from superposed relationship at some stage of said process after said image-wise distribution of dye has been transferred from said photosensitive element to said print-receiving element.

9. A process of forming images in color as defined in claim 1 including the step of mordanting, in said print-receiving material, dye which is transferred thereto.

10. A process of forming images in color as defined in claim 5 including the step of mordanting, in said print-receiving element, dye which is transferred thereto.

11. A process of forming images in color as defined in claim 1 including the step of transferring unreacted developing agent to said print-receiving material and oxidizing the transferred unreacted developing agent with an oxidizing agent distributed in said print-receiving material.

12. A process of forming images in color as defined in claim 1 wherein said developing agent is incorporated in a liquid-permeable layer of the photosensitive element and wherein said developing agent is characterized by having a molecule sufficiently large so that said developing agent will not diffuse to said image-receiving material.

13. A process of forming images in color as defined in claim 1 wherein said dye is of a color complementary to the color to which said emulsion is sensitive.

14. A process of forming images in color as defined in claim 1 wherein said developing agent is an aminophenol.

15. A process of forming images in color as defined in claim 1 wherein said developing agent is a para-phenylene diamine.

16. A process of forming images in color as defined in claim 1 wherein said dye is slowly soluble in the processing liquid and is present in the photosensitive element in a quantity in excess of that needed to provide a transfer image.

17. A process of forming images in color as defined in claim 16 including the step of forming at least one additional transfer image, after said image-receiving element and photosensitive element are separated, by again superposing said photosensitive element on an image-receiving element in the presence of a liquid capable of solubilizing said dye.

18. A photographic product comprising a photosensitive element having a liquid-permeable portion, including a photosensitive silver halide emulsion, a print-receiving element including a dyeable material for receiving a transfer image, and a container holding a liquid, said photosensitive element, said print-receiving element and said container being attached together to permit at least a portion of said print-receiving element and said photosensitive element to be superposed with said container so positioned as to be capable of being ruptured and of releasing its liquid content to at least partially permeate said superposed print-receiving element and said photosensitive element, including said emulsion, said product having positioned therein photographic processing materials, said materials including a silver halide developing agent and also including a dye which is soluble in said liquid and when dissolved therein is mobile in said photographic product, said dye possessing a coupling function capable of coupling with the oxidation product of said silver halide developing agent formed upon the development of exposed silver halide to thereby provide a reaction product which is at least sufficiently immobile in said photosensitive element so as to substantially prevent its transfer therefrom in solution in said liquid, said materials being rendered effective upon the rupture of said container for providing in said emulsion a substantially uniform distribution of said dye and said developing agent whereby to develop a latent image in said emulsion, form said reaction product which is less mobile

than said dye and provide therein an imagewise distribution comprising dye in mobile condition and transportable from said photosensitive element to said print-receiving element for imparting to the dyeable material a positive dye image having substantially the same color as said mobile dye.

19. A photographic product as defined in claim 18 wherein said developing agent is nontransferable to said image-receiving element.

20. A photographic product as defined in claim 18 wherein said coupling function of said dye is insulated from the chromophoric system of said dye by a group which prevents any system of resonance or conjugation from extending from said coupling function to said chromophoric system.

21. A photographic product as defined in claim 18 wherein at least one of said photographic processing materials is substantially uniformly distributed in a permeable layer of said photosensitive element.

22. A photographic product as defined in claim 18 wherein said developing agent is present in a permeable layer of said photosensitive element and is substantially nondiffusible to said print-receiving element from said photosensitive element in solution in said liquid.

23. A photographic product as defined in claim 18 wherein a dye mordant is substantially uniformly distributed in a stratum of said print-receiving element.

24. A photographic product as defined in claim 18 wherein at least a stratum of said print-receiving element contains a substantially uniform distribution of an oxidizing agent.

25. A photographic product as defined in claim 18 wherein said developing agent is incorporated in a liquid-permeable layer of the photosensitive element and wherein said developing agent is characterized by having a molecule sufficiently large so that said developing agent will not diffuse to said dyeable material.

26. A photographic product as defined in claim 18 wherein said dye is distributed in a stratum on said print-receiving element.

27. A photographic product as defined in claim 18 wherein said dye is of a color complementary to the color to which said emulsion is sensitive.

28. A photographic product as defined in claim 18 wherein said developing agent is an aminophenol.

29. A photographic product as defined in claim 18 wherein said developing agent is a para-phenylene diamine.

30. A photosensitive element comprising a support, at least one liquid-permeable layer mounted upon said support, photosensitive silver halide substantially uniformly distributed throughout a permeable layer of said element, a dye substantially uniformly distributed throughout a liquid-permeable layer of said element, and a silver halide developing agent substantially uniformly distributed throughout a permeable layer of said photosensitive element, said dye being soluble in a liquid processing composition and when dissolved therein being mobile in said photosensitive element, said dye possessing a coupling function capable of coupling with the oxidation product of said developing agent, and said developing agent being characterized by providing, upon the development of latent image to silver, an oxidation product reactable with said dye to provide a reaction product which is less mobile in said photosensitive ele-

ment than said dye, said reaction product being substantially nondiffusible from said photosensitive element.

31. A photosensitive element as defined in claim 30 wherein said developing agent is substantially nondiffusible from said photosensitive element.

32. A photosensitive element as defined in claim 30 wherein said coupling function of said dye is insulated from the chromophoric system of said dye by a group which prevents any system of resonance or conjugation from extending from said coupling function to said chromophoric system.

33. A photosensitive element as defined in claim 30 wherein said dye is contained in a permeable layer of the element other than the layer containing silver halide and said developing agent is contained in a permeable layer of said element other than said layer containing silver halide.

34. A photosensitive element as defined in claim 30 wherein said developing agent and said dye are both contained in the same permeable layer of said element.

35. A photosensitive element as defined in claim 30 wherein said dye is of a color complementary to the color to which said emulsion is sensitive.

36. A photosensitive element as defined in claim 30 wherein said developing agent is an aminophenol.

37. A photosensitive element as defined in claim 30 wherein said developing agent is a para-phenylene diamine.

38. A process of forming transfer images in color comprising exposing a photosensitive element including a silver halide emulsion and a dye, said dye being a dye which is capable of coupling with the oxidation product of a silver halide developing agent, said coupling being effective to displace a substituent of said dye, developing said exposed emulsion with a silver halide developing agent, coupling said dye with an oxidation product of said developing agent, forming as a function of said development an imagewise distribution of a diffusible dye and transferring at least a part of said imagewise distribution of said diffusible dye to a superposed image-receiving layer to provide a positive dye image.

39. In a diffusion-transfer process wherein an exposed photosensitive element containing a silver halide emulsion and a color-providing substance is developed, an imagewise distribution of a diffusible color-providing substance is formed as a function of said development, and said diffusible color-providing substance is transferred by diffusion to a superposed image-receiving material to impart thereto a positive dye image of a color complementary to the color to which said silver halide emulsion is sensitive, the step which comprises employing as said color-providing substance a dye which possesses a substituent displaceable upon coupling of said dye with the oxidation product of a silver halide developing agent.

#### References Cited in the file of this patent

#### UNITED STATES PATENTS

|    |           |               |       |               |
|----|-----------|---------------|-------|---------------|
| 60 | 2,306,410 | Schinzel      | ----- | Dec. 29, 1942 |
|    | 2,434,272 | Jelley et al. | ----- | Jan. 13, 1948 |
|    | 2,559,643 | Land          | ----- | July 10, 1951 |
|    | 2,698,244 | Land          | ----- | Dec. 28, 1954 |
|    | 2,704,711 | Hanson        | ----- | Mar. 22, 1955 |
| 65 | 2,756,142 | Yutzy         | ----- | July 24, 1956 |
|    | 2,774,668 | Rogers        | ----- | Dec. 18, 1956 |

UNITED STATES PATENT OFFICE  
CERTIFICATE OF CORRECTION

Patent No. 3,087,817

April 30, 1963

Howard G. Rogers

It is hereby certified that error appears in the above numbered patent requiring correction and that the said Letters Patent should read as corrected below.

Column 3, line 10, for "will" read -- with --; lines 67 and 68, for "distribu" read -- distribution --; line 70, before "formation" insert -- the --; line 74, for "serial" read -- aerial --; column 4, line 12, strike out ", now U. S. Patent No. 3,019,124" and insert the same after "1956" in line 13, same column 4; column 4, line 18, for "is" read -- in --; line 69, for "modibity" read -- mobility --; column 6, line 45, for "anthquinone" read -- anthraquinone --; column 8, line 4, for "Th.s" read -- This --; column 18, lines 49 and 50, for "soulfonate" read -- sulfonate --; line 75, for "monochromatic" read -- monochromatic --; column 21, line 11, after "from" insert -- said --; column 22, lines 41 and 42, for "addtional" read -- additional --.

Signed and sealed this 31st day of March 1964.

(SEAL)

Attest:

ERNEST W. SWIDER

Attesting Officer

EDWARD J. BRENNER

Commissioner of Patents